

# UNITED STATES PATENT OFFICE.

JOHN L. COX, OF PHILADELPHIA, PENNSYLVANIA.

## PROCESS OF MAKING PROJECTILES.

1,407,254.

Specification of Letters Patent. Patented Feb. 21, 1922.

No Drawing.

Application filed November 20, 1920. Serial No. 425,433.

To all whom it may concern:

Be it known that I, JOHN L. Cox, a citizen of the United States, residing at Philadelphia, county of Philadelphia, and State 5 of Pennsylvania, have invented a new and useful Improvement in Processes of Making Projectiles, of which the following is a full, clear, and exact description.

In the manufacture of armor piercing shot 10 and shell the necessity of combining in a projectile formed of a single block of metal a hard but not brittle head with a relatively soft and very tough body is well recognized, and projectiles having in degree such characteristics have hitherto been manufactured.

Known processes of manufacture still leave much to be desired in obtaining and combining these desirable and apparently contradictory qualities; moreover, a considerable proportion of projectiles that have 20 been subjected to recognized methods of heat treatment designed to produce the desired result fail when subjected to the rigorous ballistic tests which they must pass to be accepted.

It is the object of my invention to manufacture a projectile which will possess to a maximum degree the qualities above mentioned, and by a process which will minimize 30 the likelihood of producing any defects or weaknesses which might endanger acceptance or, later, cause spontaneous rupture in storage.

By my process a projectile is produced 35 having a point characterized by a high degree of hardness, progressively decreasing through the head toward its junction with the body, and a body sufficiently soft to permit machining yet so tough that it will not 40 break upon impact; moreover, the process is one wherein the danger of cracking during treatment is minimized, and all danger of the shell cracking in storage after delivery 45 is removed.

In the heat-treatment of steel certain laws 50 are more or less well known, but there are many conceivable ways of applying them to heat treating processes, and there is always the danger that while some of these laws 55 may be regarded others might be overlooked or ignored.

The laws that I have more especially borne in mind in the development of my process are the following:

55 1. On heating at the  $Ac_1$  point the previously existing cell boundaries of the steel

begin to disappear as the solution commences, but are not entirely gone until the  $Ac_3$  point is reached.

2. At the  $Ac_1$  point a new cell structure 60 begins to form and to grow larger as the temperature increases.

3. There is a cell size corresponding roughly to any given temperature above the  $Ac_1$  point, long maintenance at that temperature tending rather to increase the thickness of the cell boundaries than to increase 65 the cell size.

4. To acquire, on sudden cooling, the maximum hardness permitted by its chemical 70 composition steel must first be heated to or above the  $Ac_3$  point.

5. The degree of final hardness is dependent upon the speed of the quench.

6. Steel raised to a temperature much in 75 excess of the  $Ac_3$  point tends to become coarse in grain and brittle.

7. The power of hardening once acquired by steel on heating is not lost, on slow cooling, until the  $Ar_1$  point is passed. Generally 80 this temperature shows a visible color.

8. Sudden cooling from below the  $Ar_1$  point, or generally from black, theoretically will not produce hardening but the steel 85 will be in the same soft or annealed state that it would be had it been slowly cooled.

It is much less well known that on heating, sudden cooling from a point within a substantial, but limited, range below the  $Ac_1$  point as experimentally determined, 90 may produce a distinct degree of hardening and notable loss of toughness; while sudden cooling from a temperature too far below the  $Ac_1$  point to produce this effect will impart a degree of toughness superior to that 95 resulting from a slow cooling from the same or somewhat higher temperature.

It is also known to but few that the  $Ac_1$  and  $Ac_3$  points are not fixed points for any 100 particular composition but vary with the degree of grain-refinement of the steel, being lower as the grain of the steel is finer.

In my application Serial No. 311,325, filed July 16, 1919, I have described a process 105 of hardening projectiles, which process, although specifically different from the present process, has features of novelty which are also combined in the present process. Said application hence contains certain claims broadly covering the present process. In the present application I claim 110 such features of the present process as are

novel, but not disclosed in the process of said earlier application. Moreover, the process of the present application is more specifically adapted to the treatment of shells made 5 from nickel chrome shell steel (although not limited thereto) and I have used the term "black" instead of the  $Ar_1$  point, for the reason that in steel of this character the  $Ar_1$  point is frequently very difficult of determination and is sometimes unaccountably 10 low.

I shall not herein describe the process of melting the steel and casting the shell ingots.

15 After casting, the shell ingots are reheated and forged. I prefer to quench them for a few minutes to prevent grain growth, but for too short a time to produce cracking. Whether so quenched or not, they are 20 then cooled slowly until at least black throughout.

The forgings are then reheated in a continuous furnace to about  $225^{\circ}$  F. above the  $Ac_1$  temperature (generally the same as the 25  $Ac_3$  temperature in steels of this character) in order preliminarily to refine the grain. They are then removed from the furnace and cooled in the air until black throughout. The forgings are again reheated, in a second 30 continuous furnace, to a temperature of about  $75^{\circ}$  F. above the  $Ac_1$  point, to complete the refinement of the grain, and are then, in a third continuous furnace, so slowly cooled as to prevent any appreciable hardening of the steel which would interfere 35 with the preliminary machining of the shell.

After preliminary machining, the shells are reheated to considerably above the  $Ac_1$  point and quenched until well below black 40 throughout, then reheated to a less degree above the  $Ac_1$  point and quenched again until well below black, then again reheated to below the  $Ac_1$  point and quenched until well below black, followed by a slower cooling to 45 avoid unnecessary risk of cracking.

If the composition of the projectile has been properly chosen and all steps of melting, forging, and the heat-treatment described above properly applied, the projectile 50 will be in the condition of maximum toughness throughout, and soft enough readily to allow machining to finish sizes, should that step not already have been applied. It is generally advisable not to finish the band 55 score at this stage.

After further machining, the shells are ready for hardening and are heated considerably above the  $Ac_1$  point and quenched to cold; then raised to a temperature below 60  $400^{\circ}$  F. to relieve stresses, and thereafter allowed to cool.

The body of the shell is then heated close to the  $Ac_1$  point and allowed to cool and is then reheated to a temperature close to but 65 so far below the  $Ac_1$  point that no hardening

can result, and then quenched to well below black, preferably for somewhat less than the entire length and heated to avoid cracking. The shell is then inverted and placed point downward in shallow water to cool.

70 The heating and cooling of the projectile during the hardening and drawing may be carried out by any appropriate means, such, for example, as described in my above mentioned application.

75 In the foregoing steps, the first two coolings from above the  $Ac_1$  point may be made from the same temperature, but preferably the second cooling is made from a lower temperature.

80 The temperature from which the two preliminary quenches are made can be the same, but preferably the second quench is from a lower temperature than the first.

If two similar coolings or quenchings were 85 to be made from the same temperature, then the duration of the heat preceding the second cooling should be much shorter than that of the heating preceding the first cooling, to derive the full benefit from the step. 90

95 The effect of the above treatments is to impart to the head the maximum degree of hardness at the point, and a diminishing degree of hardness towards the rear without impairing the fine-grained structure of the steel, while imparting to the body the maximum degree of toughness, and a sufficient degree of softness to enable it to be readily machined if desired, as, for instance, for the attachment of the band.

100 While it is true that the elevation of the temperature of the rear of the head in the final heating operation due to the conductivity of the metal modifies somewhat its hardness, the modification is such that it 105 would be desirable to take special means to obtain it; that is, the objectionable brittleness necessarily associated with extreme hardness is largely eliminated where maximum hardness is not necessary, but there is 110 secured a maximum degree of hardness consistent with the reduction of brittleness to the desired extent. However, the amount of heat transmitted from the head to the point during the cooling of the head must be restricted to prevent diminution of the hardness of the point.

115 As it is usually dangerous to quench the whole projectile after the heating of the body, in that the projectile is likely to crack, 120 I prefer, as described above, to quench somewhat less than all the body so heated and subsequently to submerge the point in water, thereby holding down the temperature of the point.

125 I wish it to be understood that there is no clear line of demarcation between the hard and tough portions of the projectile; on the contrary, there is between the hard point and the tough body the major portion of the 130

head, shading in hardness from the point toward the body, which is not as hard as the point nor as tough as the major portion of the body.

5 The exact temperature corresponding to the  $Ac_1$ ,  $Ac_3$  and  $Ar_1$  points will vary with the composition and physical structure of the steel and the last with the degree of the latest heating and cannot be definitely 10 stated; but these points are well known to metallurgists and practical steel workers and are more informative than the specification of exact temperatures. Instruments of a number of forms exist for their accurate 15 determination. By the term "black" is meant below visible redness in the dark or a temperature of about  $950^{\circ}$  F.

Having now fully described my invention, what I claim and desire to protect by Letters Patent is:

1. The process of heat treating projectiles which comprises forging the projectile and suddenly cooling the forging to prevent grain growth but stopping the sudden cooling 25 before cracks are produced, then cooling slowly until black throughout, then reheating the projectile to about  $225^{\circ}$  F. above the  $Ac_1$  point, then cooling in the air until black throughout, then reheating to about 30  $75^{\circ}$  F. above the  $Ac_1$  point, then slowly cooling, then reheating to considerably above the  $Ac_1$  point and quenching until well below black throughout, then reheating to a less degree above the  $Ac_1$  point and quenching 35 until well below black throughout, then reheating to below the  $Ac_1$  point, quenching until well below black throughout and then more slowly cooling, then reheating to considerably above the  $Ac_1$  point and quenching 40 to cold, then heating to a temperature below  $400^{\circ}$  F. to relieve stresses and allowing to cool, then heating the body close to the  $Ac_1$  point and allowing to cool, then reheating the body portion just treated to a 45 temperature close to but so far below the  $Ac_1$  point that no hardening can result, then quenching to well below black, and then cooling the point in water and the body in air.

50 2. The process of heat treating projectiles comprising refining the grain by reheating forged projectiles to about  $225^{\circ}$  F. above the  $Ac_1$  point, then cooling in air until black throughout, then reheating to about  $75^{\circ}$  F. 55 above the  $Ac_1$  point, then slowly cooling, then reheating to considerably above the  $Ac_1$  point, then quenching until well below black throughout, then reheating to a less degree above the  $Ac_1$  point, then quenching until 60 well below black, then reheating to below the  $Ac_1$  point, quenching until well below black and then more slowly cooling; then hardening by reheating to considerably above the  $Ac_1$  point and quenching to cold;

then heating to a temperature below  $400^{\circ}$  F. 65 to relieve stresses and allowing to cool; and then toughening by heating the body close to but sufficiently below the  $Ac_1$  point to prevent hardening, then quenching to well below black, and then cooling the point in 70 water.

3. The process of heat treating projectiles comprising refining the grain by reheating forged projectiles to about  $225^{\circ}$  F. above the  $Ac_1$  point, then cooling in air until black 75 throughout, then reheating to about  $75^{\circ}$  F. above the  $Ac_1$  point, then slowly cooling in a furnace, then reheating to considerably above the  $Ac_1$  point, then quenching until well below black throughout, then reheating 80 to a less degree above the  $Ac_1$  point, then quenching until well below black, then reheating to below the  $Ac_1$  point, quenching until well below black and then more slowly cooling: then hardening by reheating to 85 considerably above the  $Ac_3$  point and quenching to cold: then de-stressing by heating to a temperature below  $400^{\circ}$  F. and allowing to cool; and then further treating the projectile to toughen the body without materially softening the point.

4. The process of heat treating projectiles comprising refining the grain by reheating forged projectiles to about  $225^{\circ}$  F. above the  $Ac_1$  point, then cooling in air until black 95 throughout, then reheating to about  $75^{\circ}$  F. above the  $Ac_1$  point, then slowly cooling in a furnace, then reheating to considerably above the  $Ac_1$  point, then quenching until well below black throughout, then reheating 100 to a less degree above the  $Ac_1$  point, then quenching until well below black, then reheating to below the  $Ac_1$  point, quenching until well below black and then more slowly cooling: and then subjecting the projectile 105 to a hardening treatment.

5. The process of heat treating projectiles which comprises cooling the forged projectile from a high temperature; then subjecting the projectile to a grain refining and 110 softening treatment including heating it to a temperature substantially above the  $Ac_1$  point and cooling slowly; and then subjecting it to a further grain refining treatment including heating to substantially above the  $Ac_1$  point and quenching, and then heating to a temperature below the  $Ac_1$  point and again quenching.

6. The process of heat treating projectiles which comprises cooling the forged projectile from a high temperature; then subjecting the projectile to a grain refining treatment including reheating to a temperature materially above the  $Ac_1$  point, then cooling in air until black, then reheating 120 to a temperature above the  $Ac_1$  point but below the temperature of the immediately preceding heat, and then cooling slowly in 125

1  
a furnace; and then subjecting the shell to a succession of heating and cooling treatments to further refine the grain.

7. The process of heat treating projectiles  
5 which comprises subjecting the projectile to heating and cooling to refine the grain, then hardening by heating to considerably above the  $Ac_1$  point and quenching to cold, then heating to below  $400^{\circ}$  F. to relieve stresses

and allowing to cool, then heating a portion 10 of the projectile from the base forward to a temperature approximating the  $Ac_1$  point, and then quenching.

In testimony of which invention, I have hereunto set my hand, at Philadelphia, Pa., 15 on this 19th day of November, 1920.

JOHN L. COX.